

Patented Sept. 7, 1926.

1,598,949

# UNITED STATES PATENT OFFICE.

WILLIAM R. WEBB, OF ROCHESTER, NEW YORK, ASSIGNOR TO EASTMAN KODAK COMPANY, OF ROCHESTER, NEW YORK, A CORPORATION OF NEW YORK.

## THE PROCESS FOR REDUCING THE VISCOSITY CHARACTERISTICS OF NITROCELLULOSE.

No Drawing.

Application filed February 11, 1925. Serial No. 8,578.

This invention relates to processes for reducing the viscosity characteristics of nitrocellulose. One object of the invention is to provide a safe, simple and inexpensive process for reducing the viscosity of nitrocellulose to the desired degree. Another object is to provide such a process in which the action is under exact control so that the results may be accurately repeated. A further object of the invention is to provide such a process in which the lowering of the viscosity characteristics may be accomplished under atmospheric pressure to avoid the trouble and expense of pressure apparatus; and may be carried out at room temperature in order to avoid needless heating expense. Another object of the invention is to lessen the time required for reducing the viscosity characteristics. Other objects will 20 hereinafter appear.

At the present time there is a demand for solutions of nitrocellulose which may be sprayed easily and yet are concentrated,—that is, they have low viscosity and contain a high percentage of nitrocellulose. But the viscosity characteristics of the usual kinds of nitrocellulose are so high that such material can not be made into the above described solutions, unless modification of it 30 is effected.

It is possible to obtain suitable kinds of nitrocellulose by modifying the conditions during the nitration of the cellulose, but it is easier and more usual to produce the kinds which have high viscosity characteristics. Moreover, the kinds of nitrocellulose which are recoverable from inexpensive waste sources, such as photographic film scrap, usually have relatively high viscosity characteristics. It is, therefore, desirable to provide a safe, simple, inexpensive, and accurately repeatable process for converting the high-viscosity types of nitrocellulose into those of low viscosity characteristics.

I have found that such a process may be carried out by treating the nitrocellulosic material with a mixture of water, acid, and a penetrant liquid. I prefer to employ a strong mineral acid, such as hydrochloric acid and to use alcohol, say ethyl alcohol, as the penetrant.

This process is applicable to nitrocellulose in various forms or associations,—such as in the form of original nitrated fibers,

or in the form of colloidized products, especially solids like pyroxylin waste and film scrap. The colloidized nitrocellulose may be associated with softeners or high boiling compounds (boiling points above 100° C.) such as camphor, butyl alcohol, etc.

The treatment may be hastened by heating the bath, even under pressure, but such troublesome refinements are unnecessary in practical operation because the process proceeds with useful rapidity at room temperature and atmospheric pressure.

While I shall now describe one embodiment of my invention, by way of illustration, it will be understood that the invention is not restricted to the details of this example, except as indicated in the appended claims. In the preferred form of my invention I use a bath comprising 40% water, 50% of ethyl alcohol and 10% of a strong mineral acid such as hydrochloric acid. Into this bath I place the nitrocellulosic material to be treated. I may immerse in it waste pyroxylin material or film scrap from which the gelatinous coatings have been removed. Undissolved nitrocellulose fibers may also be readily treated.

The time of treatment varies over a considerable range, say from several hours to several days. The end of the treatment is determined preferably by test. Representative samples of the comminuted material undergoing treatment are washed, dried, dissolved and tested for viscosity. When the end of the action is reached the bath is drained off and the materials are thoroughly washed, say in running water for several days or even a week. Washing, in warm water, say at 75° C. may be employed to hasten the purification.

The duration of the action is shorter, the stronger the acid, the more active the penetrant, the lower the original viscosity characteristics of the material undergoing treatment, and the higher the permissible viscosity characteristics in the final product.

The alcohol makes the nitrocellulose more permeable to the acid solution and thus hastens the operation, as well as causing uniform action on all parts of the material. In place of the alcohol other penetrant substances may be employed. For example, I may even use an actual nitrocellulose solvent such as methyl alcohol, care being

taken, however, that such solvent be sufficiently diluted by the water and acid to prevent dissolving of the nitrocellulose and to prevent its gumming together into masses which are difficult to handle.

In place of the hydrochloric acid I may use nitric acid for example, or a mixture of these. The percentage of acid may likewise be varied. Less than 10% acts more slowly. Above 10% the action proceeds more rapidly.

Sulphuric acid, either alone or mixed with the others is, likewise usable, although I prefer hydrochloric acid. While mineral acids act more quickly, organic acids can be used, especially in conjunction with the mineral acids. Thus acetic acid may be used as an auxiliary.

Having thus described my invention, what I claim as new and desire to secure by Letters Patent is:

1. The process of treating nitrocellulosic material which comprises acting on the same with a bath containing water, acid and a penetrant organic liquid until the viscosity characteristics of the nitrocellulose are reduced.
2. The process of treating nitrocellulosic material which comprises acting thereon with a bath containing water, mineral acid and a penetrant organic liquid at atmospheric pressure and room temperature until

the viscosity characteristics of the nitrocellulose are reduced.

3. The process of treating colloidized nitrocellulose, which comprises acting thereon with a mixture of water, mineral acid and a penetrant organic liquid until the viscosity characteristics of the nitrocellulose are reduced.

4. The process of treating solid colloidized nitrocellulose associated with a high boiling organic compound, which comprises treating the same with a mixture of water, acid and a penetrant organic liquid until the viscosity characteristics of the nitrocellulose are reduced, the percentage of penetrant being insufficient to dissolve said nitrocellulose.

5. The process of treating nitrocellulose which comprises acting thereon with a mixture of water, acid and alcohol until the viscosity characteristics of the nitrocellulose are reduced.

6. The process of treating colloidized nitrocellulose which comprises acting thereon with a mixture of water, hydrochloric acid and alcohol until the viscosity characteristics of the nitrocellulose are reduced, the percentage of alcohol being insufficient to dissolve said nitrocellulose.

Signed at Rochester, New York this 4 day of February 1925.

WILLIAM R. WEBB.